# EUROPEAN PATENT APPLICATION

(11) **EP 4 759 950 A1**
(43) Date of publication of application: **17.06.2026**
(21) Application number: 25823711.4
(22) Date of filing: 12.06.2025
(51) Int. Cl.: C22C 14/00, C22C 1/03, C22F 1/18, B21B 1/22, B21B 3/00

(54) **METHOD FOR PREPARING a-TITANIUM ALLOY SHEET HAVING HIGH DEFORMATION TWIN DENSITY**

(30) Priority: 07.08.2024 CN 202411076750
(71) Applicant: Chengdu Advanced Metal Materials Industry Technology Research Institute Co., Ltd., Chengdu, Sichuan 610300 (CN)
(72) Inventor: WANG, Liya, Chengdu, Sichuan 610300 (CN); YANG, Liu, Chengdu, Sichuan 610300 (CN); WU, Jingyi, Chengdu, Sichuan 610300 (CN); ZHONG, Yong, Chengdu, Sichuan 610300 (CN)
(74) Representative: V.O.
(86) International application number: PCT/CN2025/100612
(87) International publication number: WO 2026/031765

(57) **Abstract**

A method for preparing an α-titanium alloy plate with high deformation twin density is provided, relating to the field of titanium alloy technology, comprising: adding titanium sponge, aluminum pellets, titanium diboride, Ti-32Fe, titanium dioxide as raw materials into a smelting furnace, and performing three vacuum arc remelting operations to obtain an ingot; measuring β transus temperature T_{β} of the Ti-Al-B-based alloy by differential thermal analysis, and performing two-stage hot rolling on the ingot to obtain a slab; heating the slab to the temperature of T_{β}, holding for a first time and then water cooling, and then heating the slab to (T_{β}-200) °C, holding for a second time and then air cooling to room temperature to obtain the plate. For Ti-Al-B-based α-titanium alloy, the present application adopts a microalloying design of adding β-stabilizing element Fe, performs three vacuum arc remelting operations, and employs a process of direct rolling for cogging + two-stage hot rolling process with high pass deformation to prepare a high-density deformation twin plate, ensuring the structural uniformity of the alloy and the balance of strength and toughness at a lower cost.

## Description

This application claims priority to Chinese Patent Application No. 202411076750.7, titled "METHOD FOR PREPARING α-TITANIUM ALLOY PLATE WITH HIGH DEFORMATION TWIN DENSITY", filed on August 07, 2024 with the China National Intellectual Property Administration, which is incorporated herein by reference in its entirety.

### FIELD

The present application relates to the field of titanium alloy technology, and in particular to a method for preparing an α-titanium alloy plate with high deformation twin density.

### BACKGROUND

Ti-Al-B-based α-titanium alloy is an ideal structural material for seawater environment due to its excellent corrosion resistance, moderate strength, good plasticity and toughness, and excellent weldability. It has been widely used in various mechanical parts in the shipbuilding industry. Generally speaking, with an increase of the content of impurity elements such as Fe and O, the strength and hardness of titanium alloys increase, and the plasticity and toughness decrease significantly. Different impurity elements exhibit significantly varying degrees of influence on the strength, plasticity and toughness of Ti-Al-B-based α-titanium alloys. Therefore, the purpose of improving comprehensive mechanical properties of alloys can be achieved by reasonably controlling the content of impurity elements in the alloys.

CN115747690A discloses a method for preparing a close-packed hexagonal metal material with ultra-high-density twinned crystals. The metal material prepared by this method has ultra-high-density twinned crystals and demonstrates a significant strengthening and toughening effect. However, the invention is specifically for pure metal blocks with small dimensions and belongs to laboratory-scale fabrication, rendering it less practical in practical application fields. CN115537695A discloses a method for preparing a TB8 titanium alloy with nano-twinned crystal structure. The TB8 titanium alloy is treated with a high voltage electric pulse to obtain a nano-twinned crystal structure, achieving a good balance between its tensile strength and plasticity, thereby imparting excellent comprehensive material properties to the metastable β-type TB8 titanium alloy. However, the invention focuses on the preparation method of β-titanium alloy twinned crystals, and does not involve the preparation method of α-titanium alloy twinned crystals.

Therefore, in the conventional technology, there are requirements for improving the preparation method of the α-titanium alloy plate with high deformation twin density.

### SUMMARY

In view of the above, a purpose of embodiments of the present application is to propose a method for preparing an α-titanium alloy plate with high deformation twin density. For Ti-Al-B-based α-titanium alloy, the present application adopts a microalloying design of adding β-stabilizing element Fe, performs three vacuum arc remelting operations, and employs a process of direct rolling for cogging + two-stage hot rolling process with high pass deformation to prepare a high-density deformation twin plate, ensuring the structural uniformity of the alloy and the balance of strength and toughness at a lower cost.

Based on the above purpose, the embodiments of the present application provides a method for preparing an α-titanium alloy plate with high deformation twin density, comprising the following steps:
S1 melting: adding titanium sponge, aluminum pellets, titanium diboride, Ti-32Fe, titanium dioxide as raw materials into a smelting furnace, and performing three vacuum arc remelting operations to obtain an ingot;
S2 hot rolling: measuring the β transus temperature T_{β} of the Ti-Al-B-based alloy by differential thermal analysis, and performing two-stage hot rolling on the ingot to obtain a slab;
S3 solution and aging heat treatment: heating the slab to the temperature of T_{β}, holding for a first time and then water cooling, and then heating the slab to (T_{β}-200) °C, holding for a second time and then air cooling to room temperature to obtain the plate.

In the method, the first-stage hot rolling is direct rolling for cogging, which is carried out at a heating temperature of T_{β}+100°C for a holding time of 100-120 min, with 2-3 rolling passes, a deformation amount of ≥50% for the first pass, a deformation amount of ≥30% for the remaining passes, and rolling into a slab with a thickness of 40-55 mm; the second-stage hot rolling is carried out at a temperature of T_{β}±10°C for a holding time of 80-100 min, with 5-6 rolling passes, a deformation amount of ≥18% for each pass, a total deformation amount of ≥70% for the second-stage hot rolling, and rolling into a slab with a thickness of 5-15 mm.

In some embodiments, in S1, element addition amounts comprises by mass percentage: 3.3% ≤ [Al]% ≤ 4.8%, 0.2% ≤ [Fe]% ≤ 0.4%, 0.005% ≤ [B]% ≤ 0.007%, with the balance being titanium and inevitable impurities.

In some embodiments, the titanium sponge is grade OA titanium sponge with impurity element contents of [C]% ≤ 0.01%, [N]% ≤ 0.01%, [O]% ≤ 0.04%, [H]% ≤ 0.001%, [Fe]% ≤ 0.02%.

In some embodiments, the Ti-32Fe has impurity element contents of [C]% ≤ 0.2%, [N]% ≤ 0.1%, [O]% ≤ 0.2%, [Si]% ≤ 0.1%.

In some embodiments, in S1, in S1, a purity of the aluminum pellets is ≥ 99.7%, a purity of the Ti-32Fe is ≥ 99.8%, and a purity of the titanium dioxide is ≥ 99.5%.

In some embodiments, in S2, during the melting process, a vacuum arc remelting furnace is controlled at a vacuum pressure of ≤ 3.0Pa, an arc-stabilizing current of 5-12A, a melting voltage of 20-40V, and a melting current of 3-10kA.

In some embodiments, in S2, the ingot is subjected to peeling, end facing, and surface turning treatments.

In some embodiments, in S3, the holding time for the first-stage hot rolling is 100-120 min, and the holding time for the second-stage hot rolling is 80-100 min.

In some embodiments, in S3, the solution and aging heat treatment is performed at a heating rate of 20 °C/s.

In some embodiments, in S3, α-grains grown during the aging process have a target grain size of 20-40 µm.

The present application has at least the following beneficial technical effects:

To address the problem of poor balance between strength and toughness in the Ti-Al-B-based titanium alloy of α-titanium alloy, the present invention adopts the microalloying design of adding β-stabilizing element Fe, to improve the balance between strength and toughness of the material; performs three vacuum arc remelting operations to ensure the uniformity of compositions of the titanium alloy ingot; and employs a process of direct rolling for cogging + two-stage hot rolling process with high pass deformation to obtain a plate with a thickness of 5-15 mm, which further promotes the generation of deformation twins. The addition of Fe element changes the stacking fault energy of the alloy, thereby generating growth twins (the formation of twins is closely related to the stacking fault energy, the growth twins are rarely observed in titanium alloys, the twins in titanium alloys are generally deformation twins, and the appearance of twins can improve the mechanical properties of the alloy). The application of hot rolling process with high pass deformation further promote the generation of deformation twins.

### BRIEF DESCRIPTION OF THE DRAWINGS

In order to illustrate technical solutions in embodiments of the present application or the related technologies more clearly, drawings required for use in the embodiments or the descriptions of related technologies are briefly introduced below. Apparently, drawings described below are only some embodiments of the present application. For those skilled in the art, other embodiments can be obtained based on these drawings without creative work.
FIG. 1 is a flow chart of a method for preparing an α titanium alloy plate with high deformation twin density according to an embodiment of the present application.
FIG. 2 is a schematic diagram of a microstructure according to Example 1 of the present application.
FIG. 3 is a schematic diagram of a microstructure according to Example 2 of the present application.
FIG. 4 is a schematic diagram of a microstructure according to Example 3 of the present application.
Figure 5 is a schematic diagram of a microstructure according to Comparative Example 1 of the present application.

### DETAILED DESCRIPTION OF EMBODIMENTS

In order to make the purpose, technical solution and advantages of the present application clearer, embodiments of the present application are further described in detail in conjunction with specific embodiments and with reference to the drawings.

The terms "comprising" and "having" and any variations thereof in the specification and claims of the present application and the above-mentioned drawings are intended to cover non-exclusive inclusions. The terms "first", "second", and the like in the specification and claims of the present application or the above-mentioned drawings are used to distinguish different objects, rather than to describe a specific order. The term "plurality" means two or more, unless otherwise clearly and specifically defined.

In addition, the reference to "embodiment" in the present application means that the specific features, structures or characteristics described in conjunction with the embodiment may be included in at least one embodiment of the present application. The appearance of this phrase in various places in the specification does not necessarily refer to a same embodiment, nor is it an independent or alternative embodiment that is mutually exclusive with other embodiments. It is explicitly and implicitly understood by those skilled in the art that the embodiments described herein may be combined with other embodiments.

For Ti-Al-B-based α-titanium alloy, the present application adopts a microalloying design of adding β-stabilizing element Fe, performs three vacuum arc remelting operations, and employs a process of direct rolling for cogging + two-stage hot rolling process with high pass deformation to prepare a high-density deformation twin plate, ensuring the structural uniformity of the alloy and the balance of strength and toughness at a lower cost. Reference is made to FIG. 1, the specific method comprises the following steps:
S1 melting: adding titanium sponge, aluminum pellets, titanium diboride, Ti-32Fe, titanium dioxide as raw materials into a smelting furnace, and performing three vacuum arc remelting operations to obtain an ingot;
S2 hot rolling: measuring β transus temperature T_{β} of the Ti-Al-B-based alloy by differential thermal analysis, and performing two-stage hot rolling on the ingot to obtain a slab; and
S3 solution and aging heat treatment: heating the slab to the temperature of T_{β}, holding for a first time and then water cooling, and then heating the slab to (T_{β}-200) °C, holding for a second time and then air cooling to room temperature to obtain the plate.

In the method, the first-stage hot rolling is direct rolling for cogging, which is carried out at a heating temperature of T_{β}+100°C for a holding time of 100-120 min, with 2-3 rolling passes, a deformation amount of ≥50% for the first pass, a deformation amount of ≥30% for the remaining passes, and rolling into a slab with a thickness of 40-55 mm; the second-stage hot rolling is carried out at a temperature of T_{β}±10°C for a holding time of 80-100 min, with 5-6 rolling passes, a deformation amount of ≥18% for each pass, a total deformation amount of ≥70% for the second-stage hot rolling, and rolling into a slab with a thickness of 5-15 mm.

Furthermore, in S1, grade 0A sponge titanium, aluminum pellets (a purity of ≥ 99.7%), titanium diboride, Ti-32Fe (a purity of ≥ 99.8%) and titanium dioxide (≥ 99.5%) are used as raw materials. To address the problem of poor balance between strength and toughness in the Ti-Al-B-based titanium alloy, the method involves adding β-stabilizing element Fe to reduce the stacking fault energy of the alloy, thereby forming growth twins. Twin boundaries hinder the crack propagation, thereby improving the strength and toughness of the alloy and achieving the purpose of the coordinating the balance of the strength and toughness of the alloy. The grade OA sponge titanium is used, with impurity element contents satisfying [C]% ≤ 0.01%, [N]% ≤ 0.01%, [O]% ≤ 0.04%, [H]% ≤ 0.001%, [Fe]% ≤ 0.02%; the Ti-32Fe is used, with impurity element contents satisfying [C]% ≤ 0.2%, [N]% ≤ 0.1%, [O]% ≤ 0.2%, [Si]% ≤ 0.1%.

Furthermore, in S1, the element addition amounts comprise by mass percentage: 3.3% ≤ [Al]% ≤ 4.8%, 0.2% ≤ [Fe]% ≤ 0.4%, 0.005% ≤ [B]% ≤ 0.007%, with the balance being titanium and inevitable impurities., The raw materials are subjected to three vacuum arc remelting operations according to the above proportioning ratio. During the melting process, a vacuum arc remelting furnace is controlled at a vacuum pressure of ≤ 3.0Pa, an arc-stabilizing current of 5-12A, a melting voltage of 20-40V, and a melting current of 3-10kA to obtain an ingot of Φ250mm*300mm, which is subjected to peeling and end facing to remove oxides and impurities on the surface, and then subjected to surface turning treatment and hot processing. The vacuum arc remelting method is adopted, which demonstrates excellent capability of removing non-metallic impurities, thereby ensuring the purity and compositional uniformity of the titanium alloy ingot.

Further, in S2, the β transus temperature T_{β} of the Ti-Al-B-based alloy is measured by differential thermal analysis, the ingot is processed into a square billet with a dimension of 120-170mm*200mm*300mm, and then rolled into a slab with a thickness of 5-15 mm through two-stage hot rolling. A two-roll hot rolling test machine is used, and direct rolling for cogging is used for the first-stage heat rolling, which eliminates the forging process and saves processing costs. The first-stage heat rolling has a large deformation amount, which on the one hand can refine the grains and improve the strength of the plate, and on the other hand can provide more storage energy, to promote the generation of deformation twins, thereby improving the balance of the strength and toughness of the alloy.

Further, in S3, solution and aging heat treatment involves heating the hot-rolled slab to the temperature T_{β}, holding for 60-90 min and then water-cooling, and then heating the slab to (T_{β}-200) °C, holding for 2-4h and then air-cooling to room temperature. In some embodiments, the heat treatment is performed at a heating rate of 20 °C/s, with the temperature increasing along with the furnace. The solution and aging heat treatment process is adopted to ensure that the β phase is completely retained at room temperature during the solution treatment. Due to rapid cooling, the grains have no time to grow, thereby obtaining uniform and fine grains. The aging process allows the β phase from the solution process to decompose and precipitate slowly, which plays a role of dispersion strengthening and improves the strength of the alloy. In addition, the primary α grains slowly grow to target grain size of 20-40 µm during the aging process. The grain size is moderate, which can not only improve the strength and plasticity of the grains, but also better prevent the expansion of cracks, thereby increasing the impact toughness of the alloy.

The present application is further explained in conjunction with specific embodiments below.

### Example 1

1. Composition design: Fe element microalloying was used to improve the balance of strength and toughness of Ti-Al-B-based titanium alloy. The element addition amounts were (in mass percentage): [Al]% = 4.3%, [Fe]% = 0.25%, [B]% = 0.005%, with the balance being titanium and inevitable impurities.
2. Vacuum arc remelting: Grade 0A sponge titanium, aluminum pellets (a purity of ≥ 99.7%), titanium diboride, Ti-32Fe (a purity of ≥ 99.8%), titanium dioxide (≥ 99.5%) were used as raw materials. The materials were prepared according to the mass percentage in step 1, then subjected to three vacuum arc remelting operations. During the melting process, the vacuum arc remelting furnace was controlled at a vacuum pressure of ≤ 3.0Pa. The arc-stabilizing currents in the three vacuum arc remelting operations were 6A, 9A, and 11A respectively. The melting voltages in the melting process were 28V, 32V, and 35V. The currents in the three vacuum arc remelting operations were 5kA, 8kA, and 10kA. Ingots with dimensions of Φ250*300mm were obtained. The ingots were subjected to peeling and end facing to remove the oxides and impurities on the surface, and then subjected to surface turning treatment and hot processing.
3. Hot rolling: The β transus temperature T_{β} of the Ti-Al-B-based alloy was measured to be 994.8 °C by differential thermal analysis, and the ingots obtained in step 2 were processed into square billets with dimensions of 170mm*200mm*300mm. For the first-stage hot rolling (direct rolling for cogging), the heating temperature was 1094.8 °C, the holding time was 100 min, the number of rolling passes was 3, the deformation amount of the first pass was 50%, and the deformation amounts of the remaining passes were 30.6% and 32.3% respectively. The first-stage hot rolling had a total deformation of 76.5% and a final rolling temperature of 820 °C, and slabs with a thickness of 40mm were obtained. For the second-stage hot rolling, the heating temperature was 994.8°C, the holding time was 80min, the number of rolling passes was 6, and the deformation amounts of the 6 passes were 18%, 19.2%, 18.1%, 19.35%, 19.4%, and 18.4% respectively. The second-stage hot rolling had a total deformation of 71.25% and a final rolling temperature of 832°C, and slabs with a thickness of 11.5 mm were obtained.
4. Solution and aging treatment: The hot rolled slabs were heated to a temperature of 994.8°C and held for 60 minutes and then water-cooled, and then heated to a temperature of 794.8°C and held for 4 hours and then air-cooled to room temperature.

### Example 2

1. Composition design: Fe element microalloying was used to improve the balance of strength and toughness of Ti-Al-B-based titanium alloy. The element addition amounts were (in mass percentage): [Al]% = 4.3%, [Fe]% = 0.25%, [B]% = 0.005%, with the balance being titanium and inevitable impurities.
2. Vacuum arc remelting: Grade 0A sponge titanium, aluminum pellets (a purity of ≥ 99.7%), titanium diboride, Ti-32Fe (a purity of ≥ 99.8%), titanium dioxide (≥ 99.5%) were used as raw materials. The materials were prepared according to the mass percentage in step 1, then subjected to three vacuum arc remelting operations. During the melting process, the vacuum arc remelting furnace was controlled at a vacuum pressure of ≤ 3.0Pa. The arc-stabilizing currents in the three vacuum arc remelting operations were 6A, 9A, and 11A respectively. The melting voltages in the melting process were 28V, 32V, and 35V. The currents in the three vacuum arc remelting operations were 5kA, 8kA, and 10kA. Ingots with dimensions of Φ250*300mm were obtained. The ingots were subjected to peeling and end facing to remove the oxides and impurities on the surface, and then subjected to surface turning treatment and hot processing.
3. Hot rolling: The β transus temperature T_{β} of the Ti-Al-B-based alloy was measured to be 994.8 °C by differential thermal analysis, and the ingots obtained in step 2 were processed into square billets with dimensions of 150mm*200mm*300mm. For the first-stage hot rolling (direct rolling for cogging), the heating temperature was 1094.8 °C, the holding time was 100 min, the number of rolling passes was 2, the deformation amount of the first pass was 50%, and the deformation amount of the remaining pass was 40%. The first-stage hot rolling had a total deformation of 70% and a final rolling temperature of 803 °C, and the slabs with a thickness of 45mm were obtained. For the second-stage hot rolling, the heating temperature was 994.8°C, the holding time was 80min, the number of rolling passes was 6, and the deformation amounts of the 6 passes were 20%, 19.4%, 20.7%, 21.7%, 19.4%, and 20.7% respectively. The second-stage hot rolling had a total deformation of 74.4% and a final rolling temperature of 812°C, and the slabs with a thickness of 11.5 mm were obtained.
4. Solution and aging treatment: The hot rolled slabs were heated to a temperature of 993.1°C and held for 60 minutes and then water-cooled, and then heated to a temperature of 794.8°C and held for 4 hours and then air-cooled to room temperature.

### Example 3

1. Composition design: Fe element microalloying was used to improve the balance of strength and toughness of Ti-Al-B-based titanium alloy. The element addition amounts were (in mass percentage): [Al]% = 4.3%, [Fe]% = 0.35%, [B]% = 0.005%, with the balance being titanium and inevitable impurities.
2. Vacuum arc remelting: Grade 0A sponge titanium, aluminum pellets (a purity of ≥ 99.7%), titanium diboride, Ti-32Fe (a purity of ≥ 99.8%), titanium dioxide (≥ 99.5%) were used as raw materials. The materials were prepared according to the mass percentage in step 1, then subjected to three vacuum arc remelting operations. During the melting process, the vacuum arc remelting furnace was controlled at a vacuum pressure of ≤ 3.0Pa. The arc-stabilizing currents in the three vacuum arc remelting operations were 6A, 9A, and 11A respectively. The melting voltages in the melting process were 28V, 32V, and 35V. The currents in the three vacuum arc remelting operations were 5kA, 8kA, and 10kA. Ingots with dimensions of Φ250*300mm were obtained. The ingots were subjected to peeling and end facing to remove the oxides and impurities on the surface, and then subjected to surface turning treatment and hot processing.
3. Hot rolling: The β transus temperature T_{β} of the Ti-Al-B-based alloy was measured to be 993.1 °C by differential thermal analysis, and the ingots obtained in step 2 were processed into square billets with dimensions of 150mm*200mm*300mm. For the first-stage hot rolling (direct rolling for cogging), the heating temperature was 1093.1 °C, the holding time was 100 min, the number of rolling passes was 2, the deformation amount of the first pass was 50%, and the deformation amount of the remaining pass was 40%. The first-stage hot rolling had a total deformation of 70% and a final rolling temperature of 803 °C, and the slabs with a thickness of 45mm were obtained. For the second-stage hot rolling, the heating temperature was 993.1°C, the holding time was 80min, the number of rolling passes was 6, and the deformation amounts of the 6 passes were 20%, 19.4%, 20.7%, 21.7%, 19.4%, and 20.7% respectively. The second-stage hot rolling had a total deformation of 74.4% and a final rolling temperature of 812°C, and the slabs with a thickness of 11.5 mm were obtained.
4. Solution and aging treatment: The hot rolled slabs were heated to a temperature of 993.1°C and held for 60 minutes and then water-cooled, and then heated to a temperature of 793.1°C and held for 3 hours and then air-cooled to room temperature.

### Comparative Example 1

1. Composition design: Fe element microalloying was used to improve the balance of strength and toughness of Ti-Al-B-based titanium alloy. The element addition amounts were (in mass percentage): [Al]% = 4.3%, [Fe]% = 0.05%, [B]% = 0.005%, with the balance being titanium and inevitable impurities.
2. Vacuum arc remelting: Grade 0A sponge titanium, aluminum pellets (a purity of ≥ 99.7%), titanium diboride, Ti-32Fe (a purity of ≥ 99.8%), titanium dioxide (≥ 99.5%) were used as raw materials. The materials were prepared according to the mass percentage in step 1, then subjected to three vacuum arc remelting operations. During the melting process, a vacuum arc remelting furnace was controlled at a vacuum pressure of ≤ 3.0Pa. The arc-stabilizing currents in the three vacuum arc remelting operations were 6A, 9A, and 11A respectively. The melting voltages in the melting process were 28V, 32V, and 35V. The currents in the three vacuum arc remelting operations were 5kA, 8kA, and 10kA. Ingots with dimensions of Φ250*300mm were obtained. The ingots were subjected to peeling and end facing to remove the oxides and impurities on the surface, and then subjected to surface turning treatment and hot processing.
3. Hot rolling: The β transus temperature T_{β} of the Ti-Al-B-based alloy was measured to be 998.1 °C by differential thermal analysis, and the ingots obtained in step 2 were processed into square billets with dimensions of 150mm*200mm*300mm. For the first-stage hot rolling (direct rolling for cogging), the heating temperature was 1098.1 °C, the holding time was 100 min, the number of rolling passes was 3, the deformation amount of the first pass was 30%, and the deformation amounts of the remaining passes were 30% and 25.2% respectively. The first-stage hot rolling had a total deformation of 63.2% and a final rolling temperature of 803 °C, and the slabs with a thickness of 55mm were obtained.. For the second-stage hot rolling, the heating temperature was 998.1°C, the holding time was 80min, the number of rolling passes was 7, and the deformation amounts of the 7 passes were 20%, 20%, 19.9%, 19.9%, 19.9%, 19.9% and 20.7% respectively. The second-stage hot rolling had a total deformation of 79% and a final rolling temperature of 812°C, and the slabs with a thickness of 11.5 mm were obtained.
4. Solution and aging treatment: The hot rolled slabs were heated to a temperature of 998.1°C and held for 60 minutes and then water-cooled, and then heated to a temperature of 798.1°C and held for 3 hours and then air-cooled to room temperature.

The tensile and impact properties of the Ti-Al-B-based titanium alloy plates after solution and aging treatment in Examples 1 and 2 and the comparative example were tested, and the microstructures were observed and analyzed as shown in Table 1 and Figures 2-5. As can be seen from Figures 2-5, the titanium alloy plates prepared according to Examples 1 and 2 of the present application have the same Fe content. The twinned crystals in Example 1 has a higher content than that in Example 2, which indicates that the first-stage hot rolling with high deformation can promote the formation of twinned crystals. The plates prepared in Example 3 have a higher content of twinned crystals in the microstructure. Compared with the plates prepared in Example 2, the two types of plates have the same deformation amount, but the Fe content in Example 3 is higher. It can be inferred that the higher the Fe content, the more the content of the twinned crystals. There are almost no twinned crystals in the Comparative Example, which is attributed to the low Fe content in the plates and the insufficient deformation amount during the first-stage hot rolling in the Comparative Example. By comparing the mechanical properties of the plates in the examples and comparative examples as listed in the table, it can be seen that the higher the content of twinned crystals of the plates, the better the balance of the strength and toughness of the alloy and the more excellent the comprehensive mechanical properties.

**Table 1 Testing data of tensile properties and impact properties**

| | Example 1 | Example 2 | Example 3 | Example 4 |
|---|---|---|---|---|
| Content of Fe element, wt.% | 0.25 | 0.25 | 0.35 | 0.05 |
| Deformation of the first-stage hot rolling | 76.5% | 70% | 70% | 63.3% |
| Tensile strength (MPa) | 762 | 750 | 758 | 692 |
| Yield Strength (MPa) | 693 | 663 | 673 | 631 |
| Elongation (%) | 19.1 | 17.3 | 18.4 | 19.2 |
| Reduction of area (%) | 40.5 | 37.2 | 38.1 | 40.6 |
| Impact energy (J) | 78.6 | 72.1 | 77.5 | 45.3 |

The above are exemplary embodiments disclosed by the present application, but it should be noted that various changes and modifications can be made without departing from the scope of the disclosure of the embodiments of the present application as defined by the claims. The functions, steps and/or actions of the method claims according to the disclosed embodiments described herein do not need to be performed in any particular order. In addition, although the elements disclosed in the embodiments of the present application can be described or required in individual form, they can also be understood as plurality unless explicitly limited to the singular.

It should be understood that the singular form "a" or "an" used in the present application is intended to include the plural form unless the context clearly supports exceptions. It should also be understood that "and/or" used in the present application refers to any and all possible combinations of one or more items listed in association.

The serial numbers of the embodiments disclosed in the above embodiments of the present application are only for description and do not imply the superiority or inferiority of the respective embodiments.

Those skilled in the art should understand that the discussion of any of the above embodiments is only exemplary and is not intended to imply that the scope of the disclosure of the embodiments of the present application (including claims) is limited to these examples. Under the idea of the embodiments of the present application, the technical features in the above embodiments or different embodiments can also be combined, and there are many other changes in different aspects of the embodiments of the present application as above, which are not provided in detail for the sake of simplicity. Therefore, any omission, modification, equivalent substitution, improvement, and the like made within the spirit and principle of the embodiments of the present application should be included in the protection scope of the embodiments of the present application.

## Claims

1. A method for preparing an α-titanium alloy plate with high deformation twin density comprising:
S1 melting: adding titanium sponge, aluminum pellets, titanium diboride, Ti-32Fe, titanium dioxide as raw materials into a smelting furnace, and performing three vacuum arc remelting operations to obtain an ingot;
S2 hot rolling: measuring β transus temperature T_{β} of the Ti-Al-B-based alloy by differential thermal analysis, and performing two-stage hot rolling on the ingot to obtain a slab;
S3 solution and aging heat treatment: heating the slab to the temperature of T_{β}, holding for a first time and then water cooling, and then heating the slab to (T_{β}-200) °C, holding for a second time and then air cooling to room temperature to obtain the plate;
wherein the first-stage hot rolling is direct rolling for cogging, which is carried out at a heating temperature of T_{β}+100°C for a holding time of 100-120 min, with 2-3 rolling passes, a deformation amount of ≥50% for the first pass, a deformation amount of ≥30% for the remaining passes, and rolling into a slab with a thickness of 40-55 mm; the second-stage hot rolling is carried out at a temperature of T_{β}±10°C for a holding time of 80-100 min, with 5-6 rolling passes, a deformation amount of ≥18% for each pass, a total deformation amount of ≥70% for the second-stage hot rolling, and rolling into a slab with a thickness of 5-15 mm.

2. The method for preparing the α-titanium alloy plate with high deformation twin density according to claim 1, wherein in S1, element addition amounts comprise by mass percentage: 3.3% ≤ [Al]% ≤ 4.8%, 0.2% ≤ [Fe]% ≤ 0.4%, 0.005% ≤ [B]% ≤ 0.007%, with the balance being titanium and inevitable impurities.

3. The method for preparing the α-titanium alloy plate with high deformation twin density according to claim 2, wherein the titanium sponge is grade 0A titanium sponge, with impurity element contents of [C]% ≤ 0.01%, [N]% ≤ 0.01%, [O]% ≤ 0.04%, [H]% ≤ 0.001%, [Fe]% ≤ 0.02%.

4. The method for preparing the α-titanium alloy plate with high deformation twin density according to claim 2, wherein the Ti-32Fe has impurity element contents of [C]% ≤ 0.2%, [N]% ≤ 0.1%, [O]% ≤ 0.2%, [Si]% ≤ 0.1%.

5. The method for preparing the α-titanium alloy plate with high deformation twin density according to claim 1, wherein in S1, a purity of the aluminum pellets is ≥ 99.7%, a purity of the Ti-32Fe is ≥ 99.8%, and a purity of the titanium dioxide is ≥ 99.5%.

6. The method for preparing the α-titanium alloy plate with high deformation twin density according to claim 1, wherein in S1, during the melting process, a vacuum arc remelting furnace is controlled at a vacuum pressure of ≤ 3.0Pa, an arc-stabilizing current of 5-12A, a melting voltage of 20-40V, and a melting current of 3-10kA.

7. The method for preparing the α-titanium alloy plate with high deformation twin density according to claim 1, wherein in S2, after the two-stage hot rolling, the ingot is subjected to peeling, end facing and surface turning treatments.

8. The method for preparing the α-titanium alloy plate with high deformation twin density according to claim 1, wherein in S3, the holding time for the first-stage hot rolling is 100-120 min, and the holding time for the second-stage hot rolling is 80-100 min.

9. The method for preparing the α-titanium alloy plate with high deformation twin density according to claim 1, wherein in S3, the solution and aging heat treatment is performed at a heating rate of 20 °C/s.

10. The method for preparing the α-titanium alloy plate with high deformation twin density according to claim 1, wherein in S3, α-grains grown during the aging process have a target grain size of 20-40 µm.
